

R. J. MACDERMOTT.  
PROCESS FOR CASTING CANNON.  
APPLICATION FILED OCT. 7, 1918.

1,333,593.

Patented Mar. 9, 1920.

2 SHEETS—SHEET 1.

Fig. 1.



WITNESS

E. Johnston  
F. McGuinness

*Inventor.*  
Roger J. MacDermott

R. J. MACDERMOTT,  
PROCESS FOR CASTING CANNON,  
APPLICATION FILED OCT. 7, 1918.

1,333,593.

Patented Mar. 9, 1920.

2 SHEETS—SHEET 2.

*Fig. 2.*

*Fig. 3.*



WITNESS

E. Johnston  
F. McGuinness

*Inventor.*  
Roger J. MacDermott

# UNITED STATES PATENT OFFICE.

ROGER J. MACDERMOTT, OF SAN FRANCISCO, CALIFORNIA, ASSIGNOR TO INTERNATIONAL STEEL CORPORATION, OF SAN FRANCISCO, CALIFORNIA, A CORPORATION OF ARIZONA.

## PROCESS FOR CASTING CANNON.

1,333,593.

Specification of Letters Patent.

Patented Mar. 9, 1920.

Application filed October 7, 1918. Serial No. 257,294.

To all whom it may concern:

Be it known that I, ROGER J. MACDERMOTT, a citizen of the United States, residing at Benicia, in the county of Solano and State of California, have invented a new and useful Improvement in Processes for Casting Cannon, of which the following is a specification.

My invention relates to improvements in a process for casting cannon and the like 10 wherein a lateral binder in the shape of tubes is cast within the cannon and operates to reinforce the same against lateral strain.

The primary object of the invention is to provide an improved process for casting cannon and the like whereby a cheaper material 15 may be utilized than heretofore practicable.

It is a further object of the present invention to provide improved means for producing cannon and the like adapted to effect a 20 saving of time as well as more expensive material used in the construction thereof.

It is also an object of the present invention to provide a cast cannon having lateral binders cast integral with the body of the 25 cannon to assist in resisting lateral strains caused by the rapid expansion of combusted gases therein.

I accomplish these several features by means of the device disclosed in the drawings 30 forming a part of the present specification wherein like characters of reference are used to designate similar parts throughout said specification and drawings, and in which—

Figure 1 is a vertical sectional view of a 35 chill mold of any number of parts design or pattern prepared for casting a cannon in accordance with my improved process;

Fig. 2 is a vertical sectional view of a finished product;

Fig. 3 is a broken sectional view of a completed product; and

Fig. 4 is a transverse sectional view taken on line 4—4 of Fig. 2 in the direction indicated.

Referring to the drawings the numeral 1 45 is used to designate a chill mold having a hollow core of successively reduced portions 2 to form a cannon whose diameter will diminish in diameter from the breech to the 50 muzzle thereof.

Arranged at the top of the uppermost and largest core 2 is an enlarged portion 3 to serve as a reservoir for molten metal the purpose of which will hereinafter be more 55 fully described.

Across the top of the reservoir 3 I have placed a suitable heat insulating cover 4 to prevent the too rapid cooling of the molten metal within the mold.

Just below the cover 4 in the reservoir 3 I 60 have provided a bar 5 arranged to secure in position several tubes hereinafter described.

In the practice of my process a rifled tube 6 is first placed concentric within the mold 1 to form a core for said mold 1 and also to 65 serve as an inner sleeve or rifled barrel for the finished product.

Surrounding the tube 6 I next place in position nested perforated tubes 7 arranged in spaced relation to the core or tube 6 and 70 to each other thereby providing a series of concentric channels through which molten metal may be poured.

The tubes 6 and 7 are held in concentric position at their upper ends by means of the 75 bar 5, while the tubes are held concentrically in the mold 1 at their lower ends by means of rings 8 placed between the tubes.

In the case of cannons of larger and heavier caliber I place additional reinforcement in the shape of two imperforate tubes 9 and 10 of different lengths, the shorter one 10 preferably on the outer side so as to fill the space formed by the larger diameter or breech portion of the finished product. 85

The next step in the process is to pour molten metal into the space between the tube 6 and the chill mold 1 which metal is preferably poured between the two tubes 7 so as to prevent splashing of the molten metal while 90 being poured, said tubes 7 serving as a conduit or conveyer of such dimensions as will readily prevent splashing.

The metal flows through the apertures or perforations within the tubes 7 and fills the 95 entire mold and the reservoir 3. This surplus metal within the reservoir increases the static pressure of the molten metal so that all portions of the mold will be properly filled.

It has the further advantage that as the 100 smaller mass of molten metal near the lower portion of the mold will cool more rapidly and thereby shrink the upper and more slowly cooling portion of metal will be fed from the molten metal in the reservoir thereby providing the full quantity of metal required to produce a proper casting.

While the metal is still in a molten state the tubes 7 may be agitated laterally or longitudinally by any suitable means attached 110

to said tubes to anneal and solidify the cooling metal and thereby impart greater strength to the finished product.

The finished product will then be a cast 5 cannon having longitudinal tubes cast therein to resist lateral strain.

As the rifled core has also been cast into the cannon it is obvious that the shrinkage caused by the cooling of the poured metal 10 will cause the rifled center or barrel 6 and the tubes 7 to be securely embraced and secured to the body of the finished product.

The machine work required in rifling the core or bore may be performed previously or 15 subsequently to the casting of the cannon.

Having thus described my invention what I claim as new and desire to secure by Letters Patent is—

1. The process of casting cannon and the 20 like which consists in first placing a core or chill within a mold to form an annular channel, then placing perforated tubes within the channel and in spaced relation to the core or chill and to each other, and 25 then pouring molten metal within the mold whereby said tubes may be inclosed within the casting.

2. The step in the process of casting cannon and the like which consists in placing 30 perforated nested tubes within a cannon mold whereby said tubes may be cast within the cannon.

3. The process of casting cannon and the 35 like which consists in first placing a rifled tube within a suitable mold to form a central core for said mold, then placing perforated nested tubes around said core and in spaced relation thereto and to each other, and then

pouring molten metal into the mold to cast the tubes within the cannon.

4. The process of casting cannon and the like which consists in first placing a rifled barrel within a chill mold, having a series 45 of successive reduced portions, to form a central core therefor, then placing nested perforated tubes within the mold in spaced relation to the core and to each other to form a series of concentric channels surrounding the core, then pouring molten metal into the channels thus formed to cast 50 the tubes within the finished cannon.

5. The process of casting cannon and the like which consists in first placing a central tube within a chill mold having a reservoir arranged above the cannon portion of the 55 mold, then placing nested perforated tubes within the mold in spaced relation to each other and the central core, and then pouring molten metal into the mold and around the central core whereby said tubes may be cast 60 within a finished cannon.

6. The process of casting cannon which consists in first placing a rifled central tube within a chill mold, having a series of successive reduced portions, to form a central 65 core therefor, then placing nested perforated tubes between the core and the mold and in spaced relation to said core and to each other, then placing tubes of different lengths in the larger portions of the mold in spaced 70 relation to each other, and then pouring molten metal in the mold to cast the tubes into a finished cannon.

In witness whereof, I hereunto set my signature.

ROGER J. MacDERMOTT.